

Dec. 21, 1948.

H. CHURCH

2,456,918

DISTILLATION OF VOLATILIZABLE METALS

Filed Sept. 5, 1945



INVENTOR  
HOWARD CHURCH  
BY

*James C. Toomey  
Agt.*

## UNITED STATES PATENT OFFICE

2,456,918

## DISTILLATION OF VOLATILIZABLE METALS

Howard Church, Los Gatos, Calif., assignor to  
The Permanente Metals Corporation, Oakland,  
Calif., a corporation of Delaware

Application September 5, 1945, Serial No. 614,521

6 Claims. (Cl. 75—67)

1

This invention relates to the production of metallic magnesium; and more particularly it relates to a process for the continuous distillation of magnesium.

In the carbothermic process for the production of metallic magnesium a mixture of magnesium oxide and carbon is subjected to a temperature in the order of 2000° C. whereby magnesium and carbon monoxide are formed according to the following reaction:



Since this reaction is reversible it is necessary to cool the magnesium and carbon monoxide to a point where they are stable in the presence of each other. This cooling or chilling operation is rapidly effected with the aid of large quantities of an inert chilling medium, such as, natural gas, hydrogen, or certain of the noble gases. However, even when good chilling efficiency is achieved there is some reversion of the reaction so that the product recovered comprises a mass of about fifty per cent metallic magnesium with the remainder magnesium oxide and carbon in the ratio of about 60 to 40. There are also relatively small amounts of carbides present. The material is finely divided and the individual particles are for the most part less than one micron in size. In the industry this product is usually referred to as magnesium dust.

The refinement of this magnesium dust in order to recover solid metallic magnesium of high purity is a difficult problem. The dust is highly pyrophoric in air, apparently due to the carbides present, and must be handled in an inert atmosphere or be wet down with hydrocarbon liquid; it is not readily pelleted without the use of special equipment; and as a consequence it must be handled with considerable care and precaution.

The most widely used method for recovering solid metal from magnesium dust is a batch sublimation process wherein pellets of magnesium dust, either in dry form or wetted with liquid hydrocarbons, are introduced into a retort which is thereafter subjected to a vacuum and heated to a temperature of about 1450° F. The magnesium vaporizes and flows out of the hot section of the retort and on into a condenser chamber where it may be recovered as solid metallic magnesium. Although fair yields can be obtained by this process if sufficiently large retorts are employed, it is not economic because of the necessity to first purge the atmosphere within

2

the retort with inert gases, the difficulty of drawing a sufficiently high vacuum within the retort, the slow rate of heat transfer within the retort charge due to the poor thermal conductivity of the magnesium containing charge, the large capital investment and the high operating and maintenance costs of the apparatus used.

Continuous processes for the distillation of magnesium have never been successful. Up to the present time the art has not known any successfully operated production scale continuous distillation process. This has been due to much the same difficulties as are encountered in the batch process, particularly in so far as the heat transfer and dust handling problems are concerned. Furthermore, the continuous distillation systems of the prior art can not be operated at atmospheric pressures because it is necessary to go to temperatures which are too high for the materials of construction. It is also unsatisfactory to operate at vacuum or reduced pressure because of mechanical difficulties in achieving the desired vacuum and the condensation of magnesium in the solid state.

It is among the objects of the present invention to overcome the above difficulties and to provide a process for the continuous distillation of metallic magnesium which is economic and which can be performed readily on large scale.

These and other objects will be apparent from the description of the invention which follows:

According to the invention, a method is provided for the continuous distillation of magnesium dust or the like wherein the magnesium dust is introduced into a stream of a hot gas inert to the magnesium. The dust is entrained within the hot gases which vaporize the magnesium as the dust is propelled through the system. The temperature of the gas is not high enough to react the magnesium oxide and carbon and they remain in the solid state. The flowing mixture of gas, vapors, and solids is passed to one or more separators where a substantial proportion of the solids are removed.

Thereafter the mixture of vapors, gas, and any entrained solids, if they are present, are passed to a condenser and the magnesium is recovered in either liquid or solid form. The inert gas is readily separated for reuse or discard.

An apparatus which is particularly useful in carrying out the process of this invention is shown in the accompanying drawing entitled Fig. 1.

Referring to the drawings, a horizontally disposed elongated retort-type furnace 10 is pro-

vided, which has vertical sections 11 and 12 at each of its ends and each of which accommodate burners for heating the retort. The furnace 10 is of refractory material 13 throughout. The specific refractory materials are well-known to those skilled in the art. A vertically disposed coil 15 is located in burner section 11. This coil is preferably of a stainless steel alloy which will withstand the thermal stresses and oxidizing effects to which it will be subjected in use. The coil 15 is adapted to carry an inert gas which is introduced at a point 16 extending outside of the retort. At its upper end 17 the coil is connected to a horizontally disposed tube 18 preferably of similar material, which runs the length of the retort. Located immediately beyond the connection 17 there is a connection 19 at which point the magnesium dust to be treated is introduced from tube 14. Tube 18 terminates at the end of the retort adjacent burner section 12 and discharges into a cyclone separator 20. A pipe 21 leading from the top of separator 20 discharges into a settling chamber 22. Suitable means (not shown) are provided for the removal of the solids collected in the separator 20. Leading from the settling chamber 22 is pipe 23 which is provided with a cooling jacket 24. The pipe 23 discharges into a bag filter 25, preferably of woven glass.

In operation, hydrogen or other inert gas, such as the noble gases, helium and argon, is introduced at 16 to the coil 15 located in the burner section 11. The gas is heated to a temperature in the neighborhood of 1600° F. while it is in the coil 15. It then passes into pipe 18 and is mixed with magnesium dust entering at 19. The hot gas propels the magnesium dust through pipe 19 and during the course thereof the magnesium metal of the dust is vaporized by means of the heat supplied from the gas. The magnesium oxide and carbon are not reacted under these conditions.

As the mixture of gas, vapors and solids reach the cyclone separator 20 the solids of magnesium oxide and carbon for the most part are thrown out at the bottom of the separator, while the magnesium vapors and hydrogen gas flow over into pipe 21 and on into the collecting chamber 22 where partial condensation occurs. The remaining magnesium vapors are condensed in the cooled pipe 23 and the gas flows on to the bag filter where entrained solids are readily separated. The gas may thereafter be discarded or reused in circuit.

The system disclosed herein is adapted to operate at approximately 1600° F. and at atmospheric pressure. However, under any conditions the temperature of the carrier gas is maintained at a rate so that for any given ratio of gas to magnesium vapor the gas remains unsaturated. Advantageously, operating under normal conditions, that is at atmospheric pressure and with generally available materials, the temperature of the system should lie in a range of from 1400 to 1900° F. Higher temperatures can be employed if more highly refractory materials are employed in the apparatus. Lower temperatures can also be employed if greater quantities of carrier gas are used or if precautions are taken to seal the apparatus from the atmosphere so that it is possible to operate at reduced pressure.

Although a cyclone separator has been disclosed as the means for carrying out the separation of the vapors and gases from the solids, it is to be understood that any other means capable of performing the separation operation may also

be employed. In this connection it is to be noted that the process of this invention can be carried out in any suitable apparatus and is not intended to be limited to the embodiment disclosed herein.

There are several advantages to the process of this invention which may be apparent from the above description and which will now be pointed out.

According to the process it is possible to utilize a carrier gas for the materials to be treated which also serves as a heat transfer medium. This is a distinct advantage and eliminates many of the difficulties of previous schemes which have been proposed by the prior art. It also makes it possible to take advantage of the small particle size of the dust to obtain better heat transfer rates.

Other advantages include the ability to utilize generally available equipment which achieves considerable saving and the avoidance of the necessity for pelleting the magnesium dust which is an operation requiring special equipment. Furthermore, the dust can be employed immediately as it issues from the furnace and is separated from the chilling gas and carbon monoxide. It is unnecessary to treat it for the purpose of decreasing its pyrophoric qualities because it remains in a closed system throughout.

It is possible by judicious operation of the condensation step to control the physical state of the condensed product so as to meet the requirements for subsequent treatment or uses, i. e., it may be recovered as a solid in the form of either large or small particles as desired, or as a liquid. Any carbides present as impurities in the original dust are removed by the distillation step since they are unstable at the temperatures employed and break down to form carbon and magnesium vapor. Furthermore, no problem is encountered from sodium formed in the reduction step and it can even be recovered separately as a by-product by fractional condensation. As a consequence, the product recovered by this process is considerably less pyrophoric than the original magnesium dust.

In operations according to the process of the invention it has been possible to obtain a condensate having as much as 90 per cent magnesium when using only one cyclone separating means. When employing additional separating means in series it is possible to achieve even better separation so that for certain uses the magnesium recovered can be fabricated directly, as by extrusion or the like. Where it is desirable to use magnesium of higher purity than that obtained directly from this process, the condensed product may be refined by melting and fluxing, or batch sublimation, or otherwise. Batch sublimation is not inefficient in this case because the high magnesium content of the condensed product results in increased heat transfer during the vaporization step and increased recoveries of condensed metal.

Another significant advantage of this invention is that the solids separated from the vapors and gases comprise a mixture chiefly of magnesium oxide and carbon which has several useful purposes, particularly in compounding rubber.

This process may be used in recovering any readily volatilizable metals including sodium and 70 is not intended to be limited to the manufacture of metallic magnesium, although it is particularly advantageous in recovering the latter metal since several of the difficulties encountered with magnesium are not encountered with all other readily 75 volatilizable metals. The process is useful in re-

fining any such materials when they are of a particle size possible to be conveyed in suspension in a carrier gas.

What is claimed is:

1. In the method of refining a mixture of a volatilizable metal and less volatile solid impurity, wherein the mixture is heated to a temperature sufficient to vaporize the metal but insufficient to vaporize the impurity, and the metal vapor is separated from the unvaporized impurity, the improvement which comprises supplying at least the major portion of the heat of vaporization of the metal by means of a preheated inert gas by adding the said mixture of metal and impurity in finely divided form to the preheated gas in proportions such that a suspension of the solids in the gas is formed in which the metal at thermal equilibrium exerts a substantial partial pressure, and causing a turbulent flow of the resulting suspension thereby rapidly vaporizing the metal from the suspended solids by virtue of the heat transferred from the preheated gas to the solids suspended therein, and separating the suspended solid impurity from the gaseous mixture of inert gas and metal vapor.

2. In the method of refining a mixture of a volatilizable metal and less volatile solid impurity, wherein the mixture is heated to a temperature sufficient to vaporize the metal but insufficient to vaporize the impurity, and the metal vapor is separated from the unvaporized impurity, the improvement which comprises supplying at least the major portion of the heat of vaporization of the metal by means of a preheated inert gas by adding the said mixture of metal and impurity in finely divided form to the preheated gas in proportions such that a suspension of the solids in the gas is formed in which the metal at thermal equilibrium exerts a substantial partial pressure under a total pressure of about one atmosphere, and causing a turbulent flow of the resulting suspension thereby rapidly vaporizing the metal from the suspended solids under to total pressure of about one atmosphere by virtue of the heat transferred from the preheated gas to the solids suspended therein, and separating the suspended solid impurity from the gaseous mixture of inert gas and metal vapor.

3. The improvement of claim 2, wherein said

less volatile impurity is composed largely of the oxide of the volatilizable metal and a reducing agent capable of reducing the oxide to the metal at a high temperature, and the temperature of the mixture of inert gas and finely divided solids is well below temperatures at which substantial reduction of the oxide by the reducing agent occurs but is sufficiently high to produce substantial vaporization of the metal.

10 4. The improvement of claim 2, wherein said metal is magnesium, said impurity is composed largely of magnesium oxide and carbon, and the inert gas is preheated to about 1400° to 1900° F.

15 5. The improvement of claim 2, wherein said gas is hydrogen.

6. The method of refining a solid mixture of volatilizable metal and less volatile impurity, which comprises establishing a cyclic flow of a gas which is inert with respect to the metal, heating the gas during the course of its flow to a temperature at which the metal exerts a substantial vapor pressure but below the temperatures of substantial vaporization of said impurity, adding the solid mixture of metal and impurity in finely divided form to the flowing gas after it has been thus heated so as to cause a co-current flow of hot gas and solids suspended therein, continuing turbulent flow of the solids in gas suspension for a sufficient length of time to effect substantial heat transfer from the gas to the solids and to effect substantial vaporization of the metal, separating unvaporized solids from the gaseous mixture of metal vapor and inert gas, then condensing metal vapor from the inert gas and recycling the inert gas.

HOWARD CHURCH.

#### REFERENCES CITED

The following references are of record in the 40 file of this patent:

#### UNITED STATES PATENTS

| Number    | Name     | Date          |
|-----------|----------|---------------|
| 1,943,601 | Hansgirg | Jan. 16, 1934 |
| 2,025,740 | Hansgirg | Dec. 31, 1935 |
| 2,160,969 | Hansgirg | June 6, 1939  |
| 2,393,704 | Ogorzaly | Jan. 29, 1946 |
| 2,398,443 | Munday   | Apr. 16, 1946 |